

[54] **HIGH-TEMPERATURE, WEAR-RESISTANT COATING**

[75] Inventor: **Thomas A. Wolfla**

[73] Assignee: **Union Carbide Corporation, New York, N.Y.**

[22] Filed: **Nov. 17, 1972**

[21] Appl. No.: **307,345**

[52] U.S. Cl. .... **29/195, 117/71 M**

[51] Int. Cl. .... **B32b 15/00**

[58] Field of Search ..... **29/195 M; 117/71 M**

[56] **References Cited**

UNITED STATES PATENTS

3,705,791 12/1972 Bredzs ..... **29/195 M**

3,718,962 3/1973 Levine ..... **29/195 M**  
3,719,519 3/1973 Perugini ..... **29/195 M X**

*Primary Examiner*—L. Dewayne Rutledge

*Assistant Examiner*—E. L. Weise

*Attorney, Agent, or Firm*—Dominic J. Terminello

[57] **ABSTRACT**

A high-temperature, wear-resistant coated article, and a process for making it, comprising a substrate having a coated layer of metal oxide particles, such as  $Al_2O_3$ , substantially uniformly dispersed in a metal alloy matrix wherein said alloy comprises essentially at least one first metal selected from the group of iron, cobalt and nickel, and at least one second metal selected from the group of aluminum, silicon and chromium.

**3 Claims, No Drawings**

# HIGH-TEMPERATURE, WEAR-RESISTANT COATING

## FIELD OF THE INVENTION

This invention relates to a high-temperature, wear-resistant coated article, and a process for producing it, wherein the coated layer comprises metal oxide particles dispersed in a metal alloy matrix, said alloy matrix comprising essentially at least one first metal selected from the group consisting of iron, cobalt and nickel and at least one second metal selected from the group consisting of aluminum, silicon and chromium, with the aggregate of the first metal being at least 40% by weight and the aggregate of the second metal being between about 10% and about 40% by weight.

## BACKGROUND OF THE INVENTION

There are many excellent coatings available for providing a metal alloy substrate with a surface having specific characteristics suitable for a particular end use application. The coating may be applied to increase the wear-resistant characteristics of the substrate, decrease the contact-friction characteristics of the substrate, electrically or thermally insulate the substrate, or protect it from oxidation or other corrosive attack. For example, various types of coating materials can be applied on substrates by use of detonation guns, plasma arc devices and the like, for improving the wear resistance of the substrates. However, only a few wear-resistant coating materials can be used for high-temperature service, above 1000°F, since the physical properties and/or coefficient of thermal expansion characteristics of most of the available coating materials are not compatible with the substrates used in high-temperature environments. Complex metal alloys containing tungsten, chromium or the like, are currently being used as wear-resistant coating materials for the surfaces of superalloy turbine blades. The composition of the coating is such that the coating will form carbide phases (WC, W<sub>2</sub>C, Cr<sub>23</sub>C<sub>6</sub>) during solidification. It is these hard refractory carbides that are primarily responsible for the wear resistance of the coated surfaces. However, at high temperatures in oxygen-containing environments, the hard refractory carbide surface is consumed by oxidation. Changing the alloy composition to increase corrosion resistance is not the solution since the change usually results in decreasing the wear resistance of the coating.

Another class of wear-resistant materials that is presently used is known as cermets, and includes materials consisting of a high volume fraction (usually greater than 80%) of hard particles such as oxides, or carbides and a metallic binder. Even though the metallic binder may be relatively corrosion resistant, these materials are unsatisfactory because they lack impact and fatigue resistance. Thus a problem plaguing the industry today is combining oxidation resistance and wear resistance in a useful coating.

The present invention overcomes the above drawbacks and limitations by being directed to a coating for a substrate whereby said coating comprises a relatively low volume fraction of metal oxide particles uniformly dispersed in an oxidation-resistant metal alloy matrix.

## SUMMARY OF THE INVENTION

Broadly stated, this invention is directed to a high-

temperature, wear-resistant coated article, and process for producing it, comprising a substrate with a coated layer, said layer composed of particles of at least one metal oxide substantially uniformly dispersed in a metal alloy matrix, said alloy matrix comprising essentially at least one first metal selected from the group consisting of iron, cobalt, and nickel, and at least one second metal selected from the group consisting of aluminum, silicon and chromium, and wherein the aggregate of the first metal is at least about 40% by weight of the alloy to provide sufficient strength and ductility and the aggregate of the second metal is between about 10% and about 40% by weight of the alloy to provide sufficient corrosion resistance.

15 The coating composition of this invention in a particulate form, can be deposited on a suitable solid structural substrate by conventional plasma-spraying techniques as disclosed in U.S. Pat. Nos. 2,858,411 and 3,016,447, or by Detonation Gun techniques as disclosed in U.S. Pats. Nos. 2,714,563, 2,950,867 and 2,964,420 or by flame spraying techniques as disclosed in U.S. Pat. No. 2,861,900. The unique wear-resistant material so deposited will consist of a lamellar structure of interlocking and overlapping microscopic leaves mechanically bonded to each other and to said substrate without substantial alloying at the interface thereof, and be composed of metal oxide particles intentionally added to the oxidation-resistant metal matrix.

20 The metal oxide particles for use in this invention are selected from at least one of the group consisting of aluminum oxide, chromium oxide, beryllium oxide, titanium dioxide, silicon dioxide, thorium oxide, zirconium oxide, tantalum oxide, calcium oxide, magnesium oxide, hafnium oxide, yttrium oxide, the rare earth oxides and spinel combinations of the above such as MgO·Al<sub>2</sub>O<sub>3</sub>, NiO·Al<sub>2</sub>O<sub>3</sub> and CoO·Al<sub>2</sub>O<sub>3</sub>. The size of the metal oxide particles can vary between about 0.05 micron and about 74 microns, preferably between about 1 micron and 44 microns, and be present in a volume fraction of between about 2% and about 50%, preferably between about 5% and about 25%. Particle sizes below 0.05 micron are too small to add useful wear resistance, while sizes greater than 74 microns cause excessive wear of the mating surface. Volume fractions less than 2% do not provide sufficient wear resistance, but if the fraction is greater than 50%, the material has insufficient ductility, impact resistance and resistance to thermal fatigue. The particles, dispersed in the matrix as discrete components, must be stable in the intended high temperature operating atmosphere and substantially non-reactant with both the alloy of the matrix and the material of the substrate.

25 The metal alloy matrix of this invention comprises essentially at least one first metal selected from the group consisting of iron, cobalt and nickel, and at least one second metal selected from the group consisting of aluminum, silicon and chromium. The aggregate of the first metal should be at least 40% by weight and the aggregate of the second metal should be between about 10% and about 40% by weight. The balance of the metal alloy can be composed of one or more adventitious elements, and/or one or more elements or compounds added to impart mechanical strength and/or corrosion resistance at high temperatures; for example, tungsten, molybdenum, vanadium, manganese, carbon, rhenium, yttrium, lanthanum, boron, niobium, titanium, tantalum, zirconium and the like. The metal alloy

should be of the particulate form and sized 200 Tyler mesh and finer so that it can be mixed with the metal oxide particles prior to deposition on a suitable substrate. The metal oxide particles and the components of the metal alloy matrix material should be selected so that the metal oxide particles will not effectively react with the alloy and thereby remain substantially dispersed in the alloy matrix as discrete stable particles. In addition, the final wear-resistant coating should have a Vickers Hardness Number (VHN) of greater than 500 as determined in accordance with ASTM Test Method E92-67 using a 300 gram test load. Examples of admirably suited alloys for the matrix of this invention are shown in Table I.

Some examples of substrate materials used in various corrosive environments and admirably suited as substrates for the coating of this invention include, but are not limited to, steel, stainless steel, iron base alloys, nickel, nickel base alloys, cobalt, cobalt base alloys, chromium, chromium base alloys, refractory metals, and refractory-metal base alloys. The specific coating composition selected for a substrate intended for a particular end use environment should be selected so that it will adhere to the substrate without substantially spalling or peeling while neither the metal oxide particles nor the metal alloy matrix therein will effectively react with the substrate in its intended environment. Any artisan can determine the choice of the coating materials that can be adhesively deposited and which will be compatible with a particular selected substrate for a specified end-use environment. The deposited coating shosuld consist of discrete metal oxide particles dispersed substantially uniformly in the metal alloy matrix in a size and quantity as recited above and have a surface hardness of 500 VPN. The metal particles should be stable in the alloy matrix and the overall high-temperature, wear-resistant coating should be stable on the substrate in its intended end-use environment. Usually a coating of about 0.003 inch or thicker would be suitable for most applications.

As used herein, metal base alloy shall mean alloys wherein

alloy powder; said alloy comprising essentially at least one first metal selected from the group consisting of iron, cobalt and nickel, and at least one second metal selected from the group consisting of aluminum, silicon and chromium, the aggregate of said first metal being at least about 40% by weight and the aggregate of said second metal being between about 10% and about 40% by weight; said metal oxide particles being sized between about 0.05 micron and 74 microns and present in a volume fraction of between about 2% and about 50%; and wherein said alloy powder being sized about 200 Tyler mesh and finer; and

b. depositing said mixture of particles and powders onto a substrate by a technique selected from the group consisting of detonation gun means, plasma spraying means and flame spraying means so as to adhesively coat said substrate with a high-temperature, wear-resistant coating having a surface hardness of at least about 500 VHN.

20

EXAMPLE

A cobalt base alloy L101 having the composition shown in Table II and sized 325 Tyler mesh and finer was mixed with 30-micron size and smaller chromium oxide in various volume fractions and then deposited on JT3D turbine blades using a detonation gun under the conditions outlined in U.S. Pats. Nos. 2,714,563, 2,950,867, and 2,964,420. The blades were made of Waspaloy, a nickel base superalloy composed by weight of 1.3 Al, 3.00 Ti, 4.25 Mo, 19.50 Cr, 13.5 Co, 2.0 Fe, 0.005 B, 0.085 Zr, 0.50 Mn max., 0.75 Si max., 0.030 S max., 0.10 Cu max., 0.10 C max., and balance Ni. A  $\frac{1}{8} \times \frac{1}{4}$  inch surface of the blade known as the Z-notch was coated with the cobalt base alloy and chromium oxide mixture until a 0.008 to 0.010 inch thick layer was established. The coated blades were then tested in an engine simulator wear-test device that causes thermal stress and impact and sliding wear damage similar to an actual engine by rubbing two blade Z-notch sections against each other. The temperature in the simulator during the test was recorded at 1650°F (899°C). Due to the contact between the coated sur-

TABLE I

| Alloy Name     | Fe*  | Ni   | Co   | Total First Metal | Al   | Cr   | Si  | Total Second Metal | C    | Others                  |
|----------------|------|------|------|-------------------|------|------|-----|--------------------|------|-------------------------|
| Hastelloy X    | 18.5 | 47.3 | 1.5  | 67.3              |      | 22   | 0.5 | 22.5               | 0.10 | 0.5Mn, 0.6W, 9Mo        |
| Haynes 188     | 1.5  | 22   | 40.3 | 63.8              |      | 22   |     | 22                 | 0.08 | 0.08La, 14W             |
| Udimet 700     | 0    | 53.3 | 18.5 | 71.8              | 4.25 | 15   |     | 19.25              | 0.15 | 0.03B, 3.5Ti, 5.2Mo     |
| Inconel 718    | 18   | 53.5 |      | 71.5              | 0.6  | 19   |     | 19.6               | 0.04 | 5 Nb, 0.8Ti, 3 Mo       |
| Discaloy       | 55.8 | 26   |      | 81.8              | 0.10 | 13.5 |     | 13.6               | 0.04 | 0.005B, 1.75Ti, 2.75 Mo |
| Coast Metal 64 | 3    | 5    | 40.6 | 48.6              |      | 28   | 1   | 29                 | 0.85 | 1V, 1Mn, 19.5W          |

\* Composition in weight percent.

the base metal is present in the largest proportion by weight. High temperature shall mean 1000°F or higher. Therefore substrates to be coated according to this invention should be such that they substantially maintain their integrity at high temperatures.

The process of this invention entails the following steps:

a. preparing a mixture of at least one metal oxide selected from a group consisting of aluminum oxide, chromium oxide, beryllium oxide, silicon dioxide, titanium dioxide, thorium oxide, zirconium oxide, tantalum oxide, calcium oxide, magnesium oxide, niobium oxide, hafnium oxide, yttrium oxide, rare earth oxides, and spinel combinations of the above, with a metal

faces of two blades, a wear scar was embedded in the coated test surfaces. The depth of the wear scars in the various coating compositions tested is shown in Table III. As demonstratively shown in the test data, the addition of metal oxide particles, in various volume fractions, to the coating will substantially increase the wear resistance of the coating without degrading its good oxidation resistance.

65

TABLE II

| Composition | % by Weight   |
|-------------|---------------|
| Cobalt*     |               |
| Chromium**  | Balance<br>28 |

TABLE II-Continued

| Composition | % by Weight |
|-------------|-------------|
| Tungsten    | 19.5        |
| Nickel*     | 5           |
| Iron*       | 3           |
| Vanadium    | 1           |
| Silicon**   | 1           |
| Manganese   | 1           |
| Carbon      | 0.85        |

\* aggregate of first metal in coating — 48.65%

\*\* aggregate of second metal in coating — 29 %

nickel, and at least one second metal selected from the group consisting of aluminum, silicon and chromium, the aggregate of said first metal being at least 40% by weight of the alloy and the aggregate of said second metal being between about 10% and about 40% by weight of the alloy; the surface hardness of said coated layer being at least 500 VHN as determined using a 300 gram test load and the coated layer having a microstructure consisting of a thin lamellar structure of interlocking and overlapping microscopic leaves me-

TABLE III

| Material                                   | Depth of Wear                     | Duration of Test |
|--------------------------------------------|-----------------------------------|------------------|
| L101 alloy                                 | $1 \times 10^{-3}$ inch           | 12 hours         |
| L101 alloy + 6 v/o $\text{Cr}_2\text{O}_3$ | less than $1 \times 10^{-4}$ inch | 12 hours         |
| L101 alloy + 4 v/o $\text{Cr}_2\text{O}_3$ | $4 \times 10^{-4}$ inch           | 12 hours         |
| L101 alloy + 2 v/o $\text{Cr}_2\text{O}_3$ | $2 \times 10^{-4}$ inch           | 12 hours         |

## What is claimed:

1. A high-temperature, wear-resistant coated article comprising a solid structural substrate having a single coated layer of metal oxide particles substantially uniformly dispersed in a metal alloy matrix; at least one of said metal oxide particles selected from the group consisting of aluminum oxide, chromium oxide, beryllium oxide, calcium oxide, titanium oxide, niobium oxide, thorium oxide, zirconium oxide, tantalum oxide, silicon oxide, magnesium oxide, hafnium oxide, yttrium oxide, rare earth oxides, and the spinel combination of the above metal oxides, sized between about 0.05 micron and about 74 microns, and present in a volume fraction of between about 2% and about 50%; said metal alloy matrix comprising essentially at least one first metal selected from the group consisting of iron, cobalt and

chanically bonded to each other and to said substrate.

2. The coated article of claim 1 wherein said substrate is selected from the group consisting of steel, stainless steel, iron base alloys, cobalt, cobalt base alloys, nickel, nickel base alloys, chromium, chromium base alloys, refractory metals and refractory-metal base alloys.

3. The coated article of claim 2 wherein said metal oxide particles are selected from a group consisting of aluminum oxide, stabilized zirconium oxide and chromium oxide; said metal alloy is selected from a group consisting of nickel base alloys, iron base alloys and cobalt base alloys, and said substrate is selected from a group consisting of nickel base alloys, cobalt base alloys and iron base alloys.

\* \* \* \* \*

40

45

50

55

60

65